

- [54] DEVICE FOR LOCAL ELECTRIC-SPARK LAYERING OF METALS AND ALLOYS BY MEANS OF ROTATING ELECTRODE
- [75] Inventor: Bogomil Totev Antonov, Sofia, Bulgaria
- [73] Assignee: DSO "IZOT", Sofia, Bulgaria
- [22] Filed: Nov. 27, 1972
- [21] Appl. No.: 309,900

- [30] Foreign Application Priority Data
- Nov. 27, 1971 Bulgaria ..... 19113
- [52] U.S. Cl. ..... 219/76, 204/298
- [51] Int. Cl. ..... B23k 9/04, C23c 15/00
- [58] Field of Search ..... 204/192, 298; 219/76, 77

- [56] References Cited
- UNITED STATES PATENTS
- 3,185,814 5/1965 Rossner ..... 219/76

|           |         |                  |         |
|-----------|---------|------------------|---------|
| 3,277,266 | 10/1966 | Blaszkowski..... | 219/76  |
| 3,277,267 | 10/1966 | Blaszkowski..... | 219/76  |
| 3,446,932 | 5/1969  | Belopitov.....   | 204/192 |
| 3,546,091 | 12/1970 | Rossner .....    | 204/298 |

Primary Examiner—T. Tufariello  
Attorney, Agent, or Firm—Armstrong, Nikaido & Wegner

[57] ABSTRACT

A method is provided for local electric-spark layering of metals and alloys by means of a rotating electrode, wherein a layering electrode of rod shape and with a diameter smaller than 2 mm is rotated around its axis, said electrode being maintained from the surface to be layered at a distance in function of the disruptive voltage and the current, wherein the electrical impulses have at idle running 15 to 600 Volts and duration of from 1 to 10 microseconds. A device for accomplishing this method is also provided.

8 Claims, 7 Drawing Figures



PATENTED AUG 27 1974

3,832,514

SHEET 1 OF 2



FIG. 1



FIG. 2



FIG. 3



FIG. 4

PATENTED AUG 27 1974

3,832,514

SHEET 2 OF 2



FIG. 7



FIG. 6



FIG. 5

**DEVICE FOR LOCAL ELECTRIC-SPARK  
LAYERING OF METALS AND ALLOYS BY MEANS  
OF ROTATING ELECTRODE**

**BACKGROUND OF THE INVENTION**

The present invention relates to a method and a device for local electric-spark layering of metals and alloys by means of a rotating electrode.

Some methods are known for electric-spark layering of metals and alloys upon contact and layering on other surfaces by means of a electrode vibrating perpendicularly to the surface and moving on it.

A method is also known for electric-spark layering of metals and alloys by means of a rotating electrode, representing a disk or a brush made of the metal which is layered with radially disposed wires.

The coatings obtained according to the aforementioned methods lack uniform thickness, and suffer from the limitation of the layered area and a sufficient density. The results obtained are not reproducible and depend to a great extent to the skill of the operator. Accordingly, these methods are generally unsuited for uniform coatings on local areas which is necessary, for example, in the fields of electronics and radio engineering, which make use of relatively expensive manual devices.

Through the present invention, the aforementioned disadvantages of the known methods and devices for electric-spark layering of metals and alloys are obviated.

**DESCRIPTION OF THE INVENTION**

According to the present invention, the coating is 35 layered by means of the butt of the layering electrode, which is rodshape and having a diameter of less than 2 mm. This is accomplished by rotating the butt around its axis, supported at an optimal distance from the layered portion in function of the disruptive voltage and the current. The electrical impulses are of about 15 to about 600 volts (idle running) with a duration of 1 to 10 microseconds.

If the width of the layer is larger than the diameter of the layering electrode, for obtaining ringshaped layers as well as layers with desirable shape and dimensions, the motion of the electrode must be planetary of controllable speed and radius. In this case, it may be necessary that the layered portion must be moved planarily.

The device for the implementation of the method of the invention, contains a layering electrode, the layered portion, a generator for current impulses, a current supplying device, and an electromotor for the rotation of the layering electrode. The layering electrode is rod-shaped and under 2 mm of diameter, and is fastened to the layering head and rotated around its axis by an incorporated electromotor in the said head, which is moved with the head axially by means of a following up system. This assures an optimal distance between the butt (contact point) of the layering electrode and the fastened on the table layered portion. Both are supplied by the electrical impulses generator.

The generator of the electrical impulses should be connected with the layering electrode by means of a mercury current supplying device and the electrical impulses should be of controllable parameters: idle run-

ning voltage from 15 to 600 Volts and the duration of the impulses — from 1 to 10 microsec.

The device should posses a mechanism ensuring a planetary motion of the rotating and layering electrode 5 with controllable speed and radius to obtain coatings with a width larger than the diameter of the layering electrode or for obtaining ringshaped and other coatings. For the same scope the layering device must be equipped with a mechanism for planar moving of the table and the layered detail fastened on it by a programming facility.

The method and the device of the invention for electric-spark layering of metals and alloys, ensures the obtaining of local high quality dense coatings in a 15 programming cycle and automatic maintenance of the optimal technological parameters of the regime and high productivity.

The method and the device, according to the invention, for the electric spark layering of metals and alloys 20 will be illustrated better in terms of the drawings, wherein:

FIG. 1 represents the principles of the local electric-spark layering according to the invention;

FIG. 2 represents the principles of the local electric-spark layering by means of a rotating and planetary moving layering electrode at a radius of the planetary motion equal to the radius of the electrode;

FIG. 3 represents the principles of the local electric-spark layering of ringshaped coatings by means of the 25 rotating and planetary moving layering electrode at a radius of the planetary motion larger than the radius of the layering electrode;

FIG. 4 represents the principles of the local electric-spark layering of coatings, with a width multiply exceeding the diameter of the layering electrode.

FIG. 5 represents the block diagram of the device for 30 local electric-spark layering of metals and alloys by means of a rotating electrode;

FIG. 6 represents the schematic representation of the 35 layering head with the incorporated in it mechanism of the planetary motion of the layering electrode;

FIG. 7 represents the schematic representation of a 40 second version of the mechanism of the planetary motion of the layering electrode.

FIG. 1 shows that the layering rodshaped electrode 1 made by the layered metal or alloy performs rotational movement around its axis and its butt (contact point) is at a definite distance from the surface of the detail (part) 2. The electrical impulse generator 4 supplies the layering electrode 1 and the layered detail 2 and as a result of the electric-spark layering on the surface of the latter (the detail) a local coating is 45 formed with a form of a round platform 3, and dimensions quite near to the diameter of the layering electrode 1.

FIG. 2 shows the principle of the local electric-spark 50 layering according to the invention, by means of a electrode rotating around its axis and planetary moving 1, at a radius of the planetary motion equal to the radius of the layering electrode 1. The platform shaped coating 3 is fo a diameter equal twice the diameter of the layering electrode 1.

FIG. 3 shows the principle of the local electric-spark 55 layering of coatings by means of a rotating around its axis and planetary moving layering electrode 1, with a radius of the planetary motion larger than the radius of

the layering electrode, at which conditions the coating 3 has a form of ringshaped band.

FIG. 4 shows the principle of the local electric-spark layering of a coating, according to the invention, the width of which (the coating) substantially exceeding the diameter of the layering electrode 1, and possessing a desirable shape, obtained combining the planetary motion of the rotating layering electrode 1 and the planar displacement of the layered detail 2 by the programming facility 15 with the servomechanisms 5 and 6.

FIG. 5 shows the block diagram of the electric-spark layering device with the rotating layering electrode, according to the invention, which (the device) consists of a layering head body 7, in which on ball guidance leads axially the layering head 8, upon which is fastened the electromotor 12, to which is clamped the layering rod-shaped electrode 1 made by the layered metal or alloy. On the table 16 is fastened the layered portion 2. The layering head 8 is displaced vertically by means of the electromotor 10 and the gear mechanism 11, both guided by an electronic following up system, in such a manner that between the surface of the layered detail and the butt of the layering electrode a definite optimal gap (clearance) is maintained. The speed of the electromotor 12 is controlled by means of the device 13 in dependence of the dimensions (size) of the layering electrode 1. The electrical impulse generator 4 is coupled to the mercury current supplying device 14 and the table 16 upon which is fastened the layered portion 2. By means of the programming facility 15 and the servomechanisms 5 and 6, the table 16 and the fastened on it detail 2 is displaced and planar turned.

FIG. 6 shows one of the possible versions of the device for planetary displacement of the layering electrode 1, incorporated in the layering head. From the figure it appears that it (the device) contains a controllable electromotor 17 with a gear mechanism 18, under which (the gear mechanism) is disposed a handle carrier (clamp) with a radial (block) bearing 19, and on the shaft (axle) of the gear mechanism 18 is fastened an inverted cup 20, in which on guidances is fastened a tail piece (shank) 22 connected to the adjusting screw 21. The tail piece (shank) 22 is carrying the electromotor 12 with the layering electrode 1.

FIG. 7 shows another version of the device for planetary motion of the layering electrode 1. From the figure it appears that the device contains a controllable motor 23 with a gear mechanism 24, both disposed under the table 16 with the layered detail 2. Above the gear mechanism 24, on the shaft is fastened the framework 25, in which is disposed the body 26 with the finger 27, which axis coincides with the axis of the layering electrode 1, and the said body is led on guidances in the framework 25 and is fixed by a screw 28. The horizontally disposed connecting rod 29, carrying the body 7 of the layering head 8 is connected through a bearing upon the said finger 27 and a second finger 30, fastened upon the horizontal plate 31, led on guidance 32.

The following examples further illustrate the invention:

#### LOCAL ELECTRIC SPARK LAYERING (FIG. 5)

The layering electrode 1 rotating around its axis by means of the electromotor 12 is maintained at a optimal distance from the layered detail 2 by following up system 9 with the motor 10 and the gear mechanism 11.

The said distance is a function of the disruptive voltage and the current. The electric impulse generator 4 is coupled to the layered detail 2 directly and to the layering electrode 1 by means of the mercury current supplying device 14. The coating on the detail 2 is obtained as a result of the spark discharges. The quality of the coating for the given materials depends of the parameters of the electric impulses, the speed of the rotation of the layering electrode and the duration of the layering process, as well as of the interelectrode gap (distance), maintained by the following up system 9. At the appropriate displacement of the table 16 with the layered detail fixed on it by the mechanisms 5 and 6, controlled by the programming facility, can be obtained coatings with the desired shape and width, near to the diameter of the layering electrode 1.

#### PLANETARY MOTION OF THE LAYERING ELECTRODE (FIG. 6)

20 The controllable motor 17, by means of the gear mechanism 18 drives the cup 20, which turns the tail piece 22 and the layering electrode 1 with the rotational motor 12. By means of the screw 21 the tail piece 22 is adjusted and fixed, which determines the appropriate radius of the planetary motion. The speed of the latter (planetary motion) is controlled by the motor 17. Making use of the said device coatings 3 could be obtained, having larger width than the diameter of the layering electrode 1 and desirable shapes, as shown in 25 FIGS. 2, 3 and 4, combining the planetary motion with the respective planar displacement of the table 16 by the programming facility 15 and the servomechanisms 5 and 6.

#### PLANETARY DISPLACEMENT OF THE LAYERING ELECTRODE (FIG. 7)

35 The controllable motor 23 by means of the gear mechanism 24 drives the body 25 with the incorporated body 26 with the finger 27, which finger makes circular motion of radius preselected by the screw 28. The connecting rod 29 driven by the finger 27, drives the body 7 of the layering head 8, which with the layering electrode together performs planetary motion. This device realizes the planetary displacements of the layering electrode 1 at substantially larger radii.

40 What is claimed is:

1. A device for spark layering metals and alloys onto a substrate, said device comprising:
  - a rod shaped layering electrode;
  - first means for rotating said layering electrode about its longitudinal axis;
  - second means for moving said layering electrode in a planetary motion about its longitudinal axis;
  - table means for supporting said substrate under said electrode;
  - means for maintaining said electrode a predetermined distance from said table means wherein said distance is a function of the voltage and current applied to the electrode.
2. The device of claim 1 wherein said table means includes third means for moving said table means relative to said electrode.
3. The device of claim 1 wherein the diameter of said layering electrode is less than 2 mm.
4. The device of claim 2 wherein said first means comprises a rotational motor coupled to said layering electrode.

5. The device of claim 4 wherein said second means comprises:

- a. a shank coupled to said motor;
- b. cup means coupled to said shank;
- c. gear means coupled to said cup through block bearing means; and,
- d. motor means for driving said gear means.

6. The device of claim 5 wherein said third means comprises:

- a. servomechanisms coupled to said table means; 10 and,
- b. a program means coupled to said servomecha-

nisms.

7. The device of claim 1 wherein said first means comprises a rotational motor.

8. The device of claim 6 wherein said second means comprises:

- a. a first body coupled to said first means;
- b. a connecting rod coupled to said first body;
- c. finger means coupled to said connecting rod; and,
- d. drive means for driving said finger means in a circular motion.

\* \* \* \* \*

15

20

25

30

35

40

45

50

55

60

65